

2,975,043

TREATMENT OF DISTILLATE FUEL OILS WITH  
AQUEOUS ANTI-MICROBIAL AGENTS

Henry A. Ambrose, Penn Township, Allegheny County, Pa., assignor to Gulf Research & Development Company, Pittsburgh, Pa., a corporation of Delaware

No Drawing. Filed Dec. 30, 1955, Ser. No. 556,412

3 Claims. (Cl. 44—72)

This invention relates to treatment of distillate fuel oils with aqueous anti-microbial agents, and more particularly to treatment of distillate fuel oils that tend to deposit gels due to gel-forming microorganisms.

Numerous East Coast marketers of distillate fuel oils have, in the recent past, received growing numbers of complaints on account of malfunctioning of distillate fuel oil burners due to accumulations of gelatinous deposits in fuel lines, strainers, burner nozzles, filters, needle valves, level controls, and the like. In numerous instances physical removal of the gelatinous deposits has failed to provide more than temporary relief, with the result that further service calls have been necessary to remove additional gel deposits, often within as short a time as 7 days or less. Thus, many burner installations show a history of repeated service calls due to gel deposits within the course of a single heating season.

As an indication of the seriousness of this problem it may be noted that a recent survey of distillate fuel oil burner installations in a region where complaints due to gel deposition have been received in the past indicated that malfunctioning of the oil burners due to gel deposition might be expected at some time in the reasonably foreseeable future in two-thirds of the installations examined. Because of the novel appearance of these fuel oil gel deposits and because of their persistence in the face of ordinary methods used to combat fuel oil deposits such as sludge, and because of other factors, it has been recognized that the problem of fuel oil gels is new and distinct from previous problems of distillate fuel oil deposits.

Systematic attempts to trace the cause of fuel oil gel deposits to an entirely chemical source, such as for example, chemical impurities, degradation or decomposition of one or more of the petroleum components of the fuel oils, or to chemical additives included in the fuel oil to improve one or more of its properties, have not been successful.

It has now been found that these fuel oil gels are of microbial derivation, and that they are caused by gel-forming microorganisms in the fuel oil as such and/or in water entrained by or contacted by the fuel oil. It is my belief, based on microscopic examination of cultures of test samples, that an important source of infection of the entire distillate fuel oil production in a typical refinery is the wash-water used in aqueous refining, following distillation, of a minor proportion of the over-all distillate fuel production. It is not considered likely that the oil is contaminated prior to distillation, since the high temperatures and steam stripping to which the oil is subjected during distillation would tend to disinfect the oil. On the other hand, it has been discovered that the water used in the conventional water-washing of distillate fuel oils that have been previously treating with aqueous treating reagents, for example aqueous caustic soda (sodium hydroxide) solution, as well as the water used in preparing the aqueous treating reagents, themselves, can contain microorganisms of

the kind found in fuel oil gels and/or spores thereof. It should be noted that water that contains an extremely minute concentration of living gel-forming microorganisms or spores can constitute a very effective source of infection of distillate fuel oil, since such microorganisms exist as a substantially pure strain in distillate fuel oil and are therefore free to thrive, whereas their development is undoubtedly repressed in water due to the presence of other microorganisms and a relative scarcity of substances necessary to their existence.

The present invention is directed to a process for the reduction, at low cost, of gel deposition in the over-all refinery production of blended distillate fuel oils. The process includes the step of distilling at least two fuel oil fractions boiling in the distillate fuel oil range, one of said fractions being inferior to the other in at least one characteristic. The process further includes subjecting at least a portion of the inferior of said fuel oil fractions to an additional refining treatment involving first intimate contact thereof with a minor proportion of a liquid phase aqueous refining agent that is capable of improving the inferior characteristic of the inferior fuel oil fraction, separating the treated fuel oil fraction from the partially spent aqueous refining agent, and then water-washing the oil with wash-water, wherein the water used in at least one of said aqueous refining agent and said water-washing contains fuel oil gel-forming microorganisms. The present invention includes in combination with the foregoing procedure the steps of incorporating in the wash-water, in microbicidal proportion, an oil-insoluble anti-microbial agent that is effective to destroy gel-forming microorganisms, said incorporating being effected prior to said water-washing, and after said water-washing, separating washed, treated oil from the wash-water, and combining the washed, treated oil with the superior of said fuel oil fractions to form a blended distillate fuel oil that approximates the superior of said fuel oil fractions with respect to said characteristic and that has a reduced tendency to deposit gel due to gel-forming microorganisms.

The present invention will normally find use after fuel oil tanks and the infected fuel oil stored therein have been disinfected, although it can also be used with somewhat reduced effectiveness when storage tanks contain fuel oil that is infected with substantial proportions of gel-forming microorganisms. When used following disinfection of fuel tanks, the present invention will be useful in preventing further infection of the over-all distillate fuel oil production by disinfecting a distillate fuel oil component that is responsible to an important degree for infection with gel-forming microorganisms of the over-all refinery production of blended distillate fuel oils. By disinfecting only the wash-water used to wash that portion of the over-all distillate fuel oil production that is refined with an aqueous reagent, as opposed to disinfecting the entire supply of water used in refining the fuel oil, and/or as opposed to disinfecting the entire distillate fuel oil production, a disinfected fuel oil is produced at minimum cost. By destroying the gel-forming microorganisms before they have had a chance to multiply in the fuel oil, one can usually employ relatively lower concentrations of the anti-microbial agent.

Although the effectiveness of the present invention is in substantial part connected with the destruction of gel-forming microorganisms in the distillate fuel oil that is subjected to refining with aqueous refining agents, and in the wash-water used in conjunction therewith, before the microorganisms have had a chance to multiply and/or to infect additional fuel oil, the invention will also function to destroy gel-forming microorganisms that enter the aqueous agent-refined fuel oil subsequent to water-washing and/or that subsequently enter or that are al-

ready present in the fuel oil components with which the disinfected fraction is blended. Non-disinfected fuel oil fractions can become infected with gel-forming microorganisms, for example, by contact with infected water leaking into the oil from defective water-cooled condensers, by contact with air, or in other ways. The destruction of gel-forming microorganisms subsequent to the aqueous refining procedure is effected by the normal entrainment in the fuel oil, subsequent to water-washing, of small droplets of wash-water containing the anti-microbial agent. These water droplets will remain in the washed oil after blending with other distillate fuel oil components, where they will function to destroy gel-forming microorganisms that are contacted by said droplets, or these droplets may settle out into an aqueous layer at the bottom of the oil storage tanks, where the anti-microbial agent contained in the droplets will function to inhibit growth of gel-forming microorganisms in the aqueous layer. It is to be noted that the dispersion in the fuel oil of anti-microbial droplets will normally tend to produce a more sterile fuel oil than will treatment of the aqueous layer alone.

The fuel oil gels with which this invention is concerned have been found to occur mostly in the form of beads and films. Occasionally, however, the gel deposits are in fibrous form. The fuel oil gels have sometimes been found to be clear and yellowish in color, but more often they are dark colored, this color possibly being caused by contamination of the gel with black fuel oil sludge or other minute particles of debris normally present in the fuel oil.

Chemical analysis of a large number of samples of these fuel oil gels shows that they all contain significant proportions of water, sulfur and copper. Where the fuel oils contain chemical addition agents, such as for example sludge inhibitors, appreciable proportions of chemical components traceable to these additives, or the additives themselves, may be found in the gels. By way of illustrating the chemical composition of these gels there are presented below analytical data on two samples of fuel oil gels removed from different burner installations. In both instances the gel as such was separated from concomitant fuel oil and sediment by heating the crude sample of originally removed from the burner installation to 120° F. and then filtering through a No. 12 Whatman filter paper.

| Separated Gel                            | Gel From Burner Installation A | Gel From Burner Installation B |
|------------------------------------------|--------------------------------|--------------------------------|
| Appearance.....                          | Yellow-Green Gel.              | Black Gel.                     |
| Inspection:                              |                                |                                |
| Sulfur, Bomb, Percent.....               | 0.82.....                      | 0.73.....                      |
| Mercaptan Sulfur, Percent.....           | 0.077.....                     |                                |
| Phosphorus, Percent.....                 |                                | nil.....                       |
| Nitrogen, Percent.....                   |                                | trace.....                     |
| Water, p.p.m., Karl Fischer Method.....  | 361.....                       | 361.....                       |
| pH Value, Glass, Calomel Electrode.....  | 6.3.....                       |                                |
| Analysis, Spectrographic, p.p.m. Sample: |                                |                                |
| Aluminum.....                            | 7.....                         |                                |
| Barium.....                              | <5.....                        |                                |
| Copper.....                              | 400.....                       |                                |
| Iron.....                                | 0.6.....                       |                                |
| Magnesium.....                           | 1.....                         |                                |
| Silicon.....                             | 2.....                         |                                |
| Ash (Max. Temp. 1,000° F.), Percent..... |                                | 0.1.....                       |
| Analysis, Spectrographic:                |                                |                                |
| Aluminum.....                            |                                | trace, major.....              |
| Copper.....                              |                                | trace.....                     |
| Iron.....                                |                                | trace.....                     |
| Magnesium.....                           |                                | trace.....                     |
| Silicon.....                             |                                |                                |

The gel sample from Installation B also indicated the presence of the commercial fuel oil sludge inhibitor employed in the fuel oil. The gel sample from Installation A was not tested for the presence of sludge inhibitor.

With respect to the more significant components of the gels, the sulfur content is probably traceable directly or

indirectly to the sulfur content of the distillate fuel oil. Whether sulfur accelerates or is essential to gel deposition has not been definitely determined. However, it may be significant that the problem of gel deposition has followed the manufacture of distillate fuel oils from crude oils of relatively high sulfur content. The water content of the gels is probably traceable to moisture entrained in the fuel oil. Experimental evidence indicates that water tends to promote gel formation. The copper present in the gels appears to be traceable to copper fuel feed lines in burner installations or to the copper or brass parts of floats, valves, screens, or other copper-containing parts of the installations. Experimental evidence also indicates that copper tends to promote fuel oil gel deposits.

A systematic investigation of a large number of samples of fuel oil gels have revealed in every instance the presence of an apparently pure strain of living microorganism, and all available evidence points to these microorganisms as the cause of the fuel oil gels. It is somewhat surprising to find that any microorganisms can survive and multiply in the fuel oil, which may account, at least in part, for the apparent purity of the strain. Moreover, it has been found that a gel can be produced in incubated samples of previously sterilized fuel oil by inoculation of the fuel oil with a small amount of the gel-forming microorganisms taken from oil burner installations containing fuel oil gel deposits. It has also been found that the addition of water to the fuel oil appears to promote the development of the gels. Furthermore, when a piece of copper wire is placed in the fuel oil, gel formation appears to be promoted. Gel formation appeared to be especially favored in fuel oil samples that had been inoculated with gel-forming microorganisms and that were maintained in contact with both metallic copper and water containing organic matter capable of supporting microbial life. Whether the fuel oil gels as such are produced by the microorganisms, or whether the microorganisms or substances produced thereby merely transform fuel oil components and/or materials contained therein or contacted thereby to gel-forming materials, is not clear. The latter possibility would seem to find some support in the fact that gels resembling those found in the field have been prepared in the laboratory from a mixture of dodecyl and xylyl mercaptans and oil-soluble copper naphthenate.

Under a magnification of 430 times, the fuel oil gel-forming microorganisms appear as a mass of multicellular filaments. The filaments show branching, and there is evidence of reproduction by budding. These characteristics are typical of yeast-like microorganisms.

The exact identity of these gel-forming microorganisms is difficult to ascertain, and therefore the invention is not limited to any specific scientific class of microorganisms named herein. The fuel oil gel-forming microorganisms may be species of sulfur-utilizing filamentous bacteria of the Beggiatoaceae family, e.g., Beggiatoa, as might be suggested by the consistent presence of sulfur in the gels. However, available evidence is conflicting as to whether the fuel oil gel-forming microorganisms thrive in contact with sulfur. The possibility that the gel-forming microorganisms are of the Beggiatoaceae family would appear to be more or less negated by the fact that these gel-forming microorganisms appear under magnification as multicellular branched hyphae, and by the fact that they appear to reproduce by budding, which facts are characteristic of fungi such as Hyphomycetales, such as for example species of *Puccinillaria* or *Monilia*, i.e., *Candida*. Photomicrographs of the gel-forming microorganisms show a particularly marked similarity to those of a microorganism previously identified as a species of *Monilia*. The fact that some strains of the genus *Monilia* are known to form mucous or gelatinous masses may be significant insofar as the present problem is concerned.

As already indicated, the present invention is applicable to distillate fuel oil manufacturing procedures wherein a portion of the over-all fuel oil distillate that is relatively inferior with respect to some characteristic, for example, acidity, mercaptan sulfur, or the like, is refined with a liquid phase, aqueous treating reagent that is capable of improving the fuel oil with respect to said characteristic, and wherein treated fuel oil distillate is then separated from partially spent aqueous treating reagent and then water-washed, and wherein the water used in at least one of said aqueous treating reagent and said water-washing contains gel-forming microorganisms, and wherein following the refining of said portion of the distillate fuel oil with aqueous treating reagent, the treated, washed portion is blended with another portion of distillate fuel oil that has not been refined with said aqueous treating reagent, and that is superior to the untreated portion with respect to said characteristic, thus forming a blended distillate fuel oil that approximates the superior portion with respect to said characteristic, and that has a reduced tendency toward gel-deposition. For example, the method of reducing gel-deposition disclosed herein will be useful when used in conjunction with the water-wash that follows aqueous caustic soda refining of distillate fuel oil that has a relatively high acid number due to the presence of a relatively large proportion of acidic substances, such as naphthenic acids. An example of a distillate fuel oil having a high acid number is a straight run fuel oil distillate obtained from a crude oil produced in Southern Louisiana. A total acid number of 0.2, which is above typical manufacturing specifications, is not unusual in such distillate.

In the neutralization of distillate fuel oils that have high acid numbers with aqueous caustic soda, the acidic fuel oil distillate is normally contacted with a quantity of caustic soda, in aqueous solution, which is greater than that theoretically required to neutralize the acidic substances in the oil. After the caustic soda contacting is complete, partially spent caustic soda solution, that is, caustic soda solution of reduced basicity, is separated from the neutralized oil and the latter is then washed with water to remove dissolved salts, soaps, and entrained caustic soda solution.

Aqueous caustic soda refining is also useful in reducing the mercaptan content of distillate fuel oils, whether or not the caustic treating is carried out in conjunction with a mercaptan solutizer or extracting agent, such as sodium isobutyrate, and the herein disclosed method of reducing gel deposition in distillate fuel oils is useful in such processes when combined with the water-wash that conventionally follows separation of partially spent caustic from aqueous caustic soda treated fuel oil. In such processes, acidic substances such as naphthenic acids will also be neutralized by the caustic soda treatment.

In any event, the refining of distillate fuel oils with liquid phase, aqueous caustic soda solution, either for the purpose of reducing the acid number of the fuel oil, and/or for the purpose of extracting mercaptans, is conventional. In general, such processes are carried out by contacting the distillate fuel oil with about 2 to about 20 percent by volume of about 2° to 40° Bé. aqueous caustic soda at atmospheric pressure and at temperatures between ambient atmospheric temperature and 210° F. Any conventional mixing apparatus designed to produce a high degree of intermixiture of immiscible liquids can be used in the caustic soda contacting. For example, there can be used a vessel adapted for countercurrent flow and containing a system of baffles. The use of strong caustic soda solution, e.g., 35° Bé., is not uncommon, especially where emulsification during water-washing is not severe, but rather dilute caustic soda solution of about 2° to 10° Bé. is often preferred in order to obtain a high degree of contact with the oil. Elevated temperatures are often desirable, since they tend to facilitate separation of the oil from partially spent caustic soda solution. Following

contact of the oil with aqueous caustic soda solution, partially spent caustic soda solution is separated by gravity settling, centrifuging or other equivalent conventional means designed to utilize differences in densities and the substantial immiscibility of the materials being treated.

After separation of neutralized oil, the neutralized oil is then water-washed in either a single stage or a plurality of stages, usually with about 10 to 200 volume percent water, to remove inorganic salts, soaps, and entrained, partially spent caustic soda solution. Any conventional apparatus, adapted for either countercurrent or concurrent flow that is designed to obtain a high degree of intercontact, can be used for said water-washing. For example, spray-washing can be used. In this method, water is added to the oil in fine streams without agitation; as the individual drops are relatively large, they tend to settle quickly. The spray is continued until a large portion of the soaps, salts, etc. are removed from the oil.

Notwithstanding the unusual effectiveness of the present invention in conjunction with aqueous caustic soda refining of distillate fuel oils, the present invention is not solely applicable to such refining procedures, but it can also be used in other liquid phase aqueous refining procedures that are terminated by water-washing. An example of a distillate fuel oil refining procedure involving aqueous treating reagents, other than aqueous caustic soda, is the doctor sweetening process wherein "sour," that is, mercaptan-containing, fuel oils are "sweetened" by converting the mercaptans to alkyl disulfides. According to conventional plant practice, sour fuel oil is sweetened by contact with about 1 to 2 volume percent of doctor solution, at atmospheric pressure and at temperature ranging from ambient atmospheric temperature to about 210° F. Elemental sulfur, in an amount sufficient to convert the lead mercaptides produced during the sweetening process to alkyl disulfides and lead sulfide, but not more than about 10 to 20 percent in excess of this amount, is provided in the sweetening reaction. The elemental sulfur may be furnished to the reaction in part or entirely from the elemental sulfur content of the fuel oil or from an external source. It is normally considered the better practice to add elemental sulfur to the sour oil before contact thereof with doctor solution. Doctor solution, as is known, comprises sodium plumbite, which can be conveniently prepared by approximate saturation of an aqueous caustic soda solution, usually about 6 to 30° Bé., with litharge. After the sweetening reaction is complete, the partially spent doctor solution is separated from the sweetened oil, and the latter is washed with water, usually 10 to 200 volume percent, to remove partially spent doctor solution, salts and other water-soluble materials. Contacting methods, conditions and apparatus for doctor treating are similar to those used for aqueous caustic soda refining.

In the application of the herein disclosed method of reducing gel deposition to the aqueous refining of distillate fuel oils, an oil-insoluble anti-microbial agent that is effective to destroy the fuel oil gel-forming microorganisms will be dissolved in microbicidal proportions in the water used in the water-washing of the distillate fuel oil that has been refined with an aqueous treating reagent. Since the aqueous refining procedures to which this invention is applicable include subsequent water-washing, the use of an anti-microbial agent of the kind disclosed herein in the wash-water will be effective not only to reduce contamination of the fuel oil with gel-forming microorganisms resulting from contact with said wash-water, but also such use will be effective to destroy any gel-forming microorganisms that have contaminated the fuel oil during some earlier stage of the refining process, for example during the prior contact of the oil with aqueous caustic soda solution, doctor solution, or the like.

The use of an anti-microbial agent of the kind disclosed herein in the wash-water is advantageous in that such use substantially avoids any problems of chemical compatibility and/or of reduced effectiveness of the anti-microbial agent due to adverse effects of the fuel oil treating reagent thereon. Moreover, the use of the anti-microbial agent in the wash-water only, rather than also in the water used in preparing the aqueous treating reagent, or in the entire water supply, minimizes the cost of effectively treating the aqueous agent-refined distillate fuel oil to reduce gel deposition therein.

As has been heretofore indicated, the present invention is confined to treating of distillate fuel oils that are subjected to aqueous refining. This is advantageous in that treatment according to this invention is restricted to that portion of the fuel oil that is contaminated with gel-forming microorganisms, and which, if not treated to destroy such microorganisms before blending with other distillate fuel oil components that have not been refined with liquid phase aqueous reagents, would act as a source of contamination for the entire refinery production of distillate fuel oil. It is, of course, unnecessary in conventional refinery practice to subject all of the distillate fuel oil production to aqueous refining procedures of the type disclosed herein. Rather, it is customary merely to treat that fraction of the total refinery production of distillate fuel oil that does not meet manufacturing specifications with respect to some characteristic that can be improved by the aqueous refining agent. For example, only that portion of fuel oil distillate that has an acid number or mercaptan content above specification limits, or so much of that portion as is necessary to treat in order for the blended product to have satisfactory properties, will be subjected to aqueous caustic soda contacting.

As previously indicated, according to my invention, the portion of over-all refinery product of distillate fuel oil that has been refined with an aqueous treating reagent and that has been washed with water containing a microbicidal proportion of an anti-microbial agent effective to destroy gel-forming microorganisms, is blended with additional distillate fuel oil that has not been refined with the aqueous treating agent and water-washed, in order to produce a blended distillate fuel oil that approaches said additional distillate fuel oil with respect to the characteristic that has been improved by aqueous refining, and that exhibits reduced tendencies toward gel-deposition due to gel-forming microorganisms. It is again noted that distillate fuel oils that are exposed to gel-forming microorganisms after treatment according to this invention, whether or not they have been blended with other fuel oil components, will possess reduced gel-forming tendencies because of the carry-over in such oils of droplets of wash-water that contain an anti-microbial agent.

Anti-microbial agents that are suitable for the purposes of this invention are those that are capable of destroying or killing the fuel oil gel-forming microorganisms, that are substantially insoluble in the distillate fuel oil that is treated thereby, and that can be dissolved in water. An example of an anti-microbial agent that has been found to be especially effective for the purposes of this invention, particularly in conjunction with aqueous caustic soda refining processes, is the sodium salt of 2,4,5-trichlorophenol, marketed under the name "Dowicide B" by the Dow Chemical Company. Dowicide B is soluble in water in the proportion of 113 grams per 100 grams of water at 25° C., and it is only slightly soluble in No. 2 fuel oil. This agent has been found effective to destroy gel-forming microorganisms in concentrations as low as one part in 80,000. Other water-soluble, substantially fuel oil-insoluble anti-microbial agents which have been found effective for the purposes of this invention are mixed alkyltolylmethyl-trimethylammonium chlorides containing alkyl groups ranging from  $C_9H_{19}$  to  $C_{15}H_{31}$  (marketed as "Hyamine 2389" by Rohm & Haas) and

mixed alkylidimethylbenzylammonium chlorides wherein the alkyl groups are  $C_8H_{17}$  to  $C_{18}H_{37}$  (marketed as "Roccal" by Sterwin Chemical Company). Hyamine 2389 and Roccal have been found effective when used in concentrations respectively of one part in 80,000 and one part in 10,000. However, the invention is not limited to the use of the above-specified anti-microbial agents, and other anti-microbial agents capable of killing gel-forming microorganisms, that are substantially insoluble in distillate fuel oil, and that can be dissolved in water, can be used. Although the action of the anti-microbial agents upon the gel-forming microorganisms with which this invention is concerned is selective, other suitable anti-microbial agents can be determined by means of suitable 10 laboratory scale tests. According to one suitable test, there is first prepared a solution containing the anti-microbial agent that is to be tested, usually one part of the anti-microbial agent (by weight, if solid; by volume, if liquid) per 100 parts of water. To a nutrient medium 15 capable of supporting the growth of the gel-forming microorganisms there is then added a quantity of the solution of the anti-microbial agent that will produce the desired test concentration of anti-microbial agent in the resulting mixture. A commercial nutrient medium, 20 marketed as Mycophyl Broth, by the Baltimore Biological Laboratories, has been found effective to support growth of the gel-forming microorganisms. This material is a solution of polypeptone and dextrose having a pH of 7. The resulting solution of anti-microbial agent in the nutrient 25 medium is then inoculated with a stock culture of gel-forming microorganisms. The resulting mixture is then incubated at 20° C. for 60 days. If the microorganisms show no evidence of growth after 60 days, the agent is regarded as effective, in the concentration 30 tested, for use in the process disclosed herein. However, in order to increase contact of microorganisms and anti-microbial agents, and/or in instances where the effectiveness of the anti-microbial agent tends to be reduced by the traces of spent aqueous refining agent, soaps or salts 35 in the wash-water, it may be desirable to employ concentrations of the anti-microbial agent that are from two to four times as great as those indicated as useful by the above-described test.

The addition of small amounts of anti-microbial agents 40 of the type disclosed herein to the wash-water used in washing distillate fuel oils that have been subjected to aqueous refining will ordinarily produce satisfactory results. The anti-microbial agents of this invention should be used in concentrations that are effective to 45 destroy the gel-forming microorganisms, i.e., in microbicidal proportion. The optimum concentration of the anti-microbial agents of this invention may, of course, vary with the nature of the individual agents themselves and possibly in some instances according to the degree of 50 infection of the fuel oil, and/or the water used in aqueous refining thereof, with gel-forming microorganisms. In general, within these limits, effective results will be obtained by dissolving in the wash-water anti-microbial agents of the kind disclosed herein in amount of between 55 about 0.001 and about 0.1 percent. Normally, concentrations of about 0.005 to about 0.05 will be preferred so as to obtain a good balance between economy and effectiveness of results. However, in individual instances, 60 for example, those where the water used in aqueous refining of the fuel oil involves a relatively low degree of infection of gel-forming microorganisms and/or relatively highly effective anti-microbial agents, concentrations of 65 anti-microbial agents as low as 0.001 percent, or possibly even less, can be used. On the other hand, in other instances, for example, where the water used in aqueous refining involves a relatively high degree of infection and/or a relatively less active anti-microbial agent, concentrations of anti-microbial agent of 0.1 percent, or 70 possibly more, may be desirable.

Fuel oils that can be treated according to this invention are those distillate fuel oils that tend to deposit gels due to the presence of gel-forming microorganisms and that are subjected to refining with an aqueous treating reagent and wash-water, at least one of which contains gel-forming microorganisms. A specific example of a fuel oil, the treatment of which is included by this invention, is No. 2 fuel oil, a type of distillate fuel used for domestic heating and light industrial heating purposes. A No. 2 fuel oil is defined in the ASTM Standards on Petroleum Products and Lubricants, under the specification designated D-396-48T. Specific examples of other distillate fuel oils included by the invention are diesel fuels and No. 1 fuel oil. It is noted that the problem of gel formation due to microorganisms appears to be restricted to distillate fuel oils. The reason for this apparent selectivity is not certain, but it may be due to the characteristically high sulfur content of these fuel oils, or it may be due to the nature of the conditions under which these oils are used. Thus, these oils are normally used in installations involving relatively long term storage in contact with water and copper.

The terms "microbial," "anti-microbial," "microbicial" and the like are used herein in their broader sense and as such have reference to microbes or microorganisms generally, whether or not they are pathogenic.

*Example*

In a specific embodiment of the herein disclosed invention, 13,000 barrels per day of a catalytically cracked No. 2 fuel oil distillate boiling between about 350° and 650° F., and having a total acid number of about 0.1, is pumped, following distillation, to a blending tank, together with 2,000 barrels per day of a South Louisiana straight run No. 2 fuel oil distillate boiling in the same range and having a total acid number of 0.21. Five thousand barrels per day of the same South Louisiana straight run fuel oil distillate is passed while still warm from distillation into a caustic contactor where it is intimately contacted at atmospheric pressure with aqueous caustic soda solution, at ambient temperature, in the proportion of 640 barrels per day. The caustic soda solution is made up by diluting 11° Bé. caustic soda concentrate with water that contains gel-forming microorganisms in the ratio of 40 barrels of caustic concentrate (11° Bé.) for every 600 barrels of water. The mixture of neutralized distillate fuel oil and partially spent caustic soda solution is removed from the caustic contactor to a settling tank. Partially spent caustic soda solution is withdrawn from the bottom of the settling tank. Neutralized fuel oil distillate is withdrawn from the top of the settling tank and spray-washed, at atmospheric pressure, and at ambient temperature, with 1667 barrels per day (33.3 volume percent) of the same water that was used to dilute the caustic soda concentrate, but to which there has been added a 10 percent aqueous solution of the sodium salt of 2,4,5-trichlorophenol at the rate of 35 gallons per day. After water-washing, the washed fuel oil is allowed to settle, whereupon separated water is drawn off, and the neutralized, washed oil, containing entrained droplets of water that in turn contain dissolved sodium salt of 2,4,5-trichlorophenol, is blended with the catalytically cracked No. 2 fuel oil and the unneutralized South Louisiana straight run No. 2 fuel oil distillate referred to previously. According to the procedure described, 20,000 barrels per day of No. 2 fuel oil distillate having a total acid number of about 0.1 and having a substantially reduced tendency to deposit gels will be produced.

The foregoing example is illustrative only and other procedures involving refining of distillate fuel oils with aqueous treating reagents and water-washing of a portion of the over-all refinery production of distillate fuel oil can be adapted to the present invention. For example, in place of the South Louisiana straight run fuel

oil distillate of the foregoing example there can be substituted an objectionably sour West Texas straight run fuel oil distillate, and for the aqueous caustic soda there can be substituted 2 percent by volume of doctor solution prepared by dissolving 1.5 percent litharge in a 16° Bé. sodium hydroxide solution. In place of the sodium salt of 2,4,5-trichlorophenol there can be substituted equivalent proportions of mixed  $C_{9-15}$  alkyltolyltrimethylammonium chlorides and mixed  $C_{8-18}$  alkyldimethylbenzylammonium chlorides.

Obviously many modifications of the invention hereinabove described may be made without departing from the spirit and scope thereof, and therefore only such limitations should be imposed as are indicated in the claims appended hereto.

I claim:

1. A process for refining distillate fuel oil, comprising providing at least two fuel oil fractions boiling in the distillate fuel oil range, one of said fractions being inferior to the other in at least one characteristic that can be improved by aqueous refining, subjecting at least a portion of the inferior of said fuel oil fractions to an aqueous refining treatment comprising first, intimate contact thereof with a minor proportion of a liquid phase aqueous refining agent that is capable of improving the inferior characteristic of the inferior fuel oil fraction, separating the treated fuel oil fraction from the partially spent aqueous refining agent, and then water-washing the oil with wash-water to remove water-soluble substances from the treated oil, wherein the water used in at least one of said aqueous refining agent and said water-washing contains fuel oil gel deposit-forming microorganisms, and prior to said water-washing, incorporating in the wash-water, in microbicial proportion, an oil-insoluble, anti-microbial agent that is effective to destroy said gel deposit-forming microorganisms under conditions of pH, temperature and nutrition favorable to their growth, and after separation of the washed, treated oil from wash-water, blending the washed, treated oil with the superior of said fuel oil fractions to form a blended distillate fuel oil that approximates the superior of said fractions with respect to said characteristic, and that has a reduced tendency to deposit gel due to gel deposit-forming microorganisms.
2. A process for refining distillate fuel oil, comprising providing at least two fuel oil fractions boiling in the No. 2 fuel oil range, one of said fractions being inferior to the other in at least one characteristic that can be improved by aqueous refining, subjecting at least a portion of the inferior of said fuel oil fractions to an aqueous refining treatment comprising first, intimate contact thereof with about 1 to 20 percent by volume of an aqueous alkaline solution of an inorganic refining agent that is capable of improving the inferior characteristic of the inferior fuel oil fraction, separating the treated fuel oil fraction from the partially spent aqueous alkaline solution of said inorganic refining agent, and then water-washing the oil with 10 to 200 volume percent wash-water to remove water-soluble substances from the treated oil, wherein the water used in at least one of said aqueous alkaline solution and said water-washing contains fuel oil gel deposit-forming microorganisms, and prior to said water-washing, incorporating in the wash-water, in a microbicial proportion of about 0.001 to 0.1 percent, an oil-insoluble, anti-microbial agent that is effective to destroy said gel deposit-forming microorganisms, said agent being selected from the group consisting of the sodium salt of 2,4,5-trichlorophenol, alkyltolyltrimethylammonium chlorides whose alkyl groups contain 9 to 15 carbon atoms, and alkyltrimethylbenzylammonium chlorides whose alkyl groups contain 8 to 18 carbon atoms, and after separation of the washed, treated oil from wash-water, blending the washed, treated oil with the superior of said fuel oil fractions to form a blended distillate fuel oil that approximates the superior

of said fractions with respect to said characteristic, and that has a reduced tendency to deposit gel due to gel deposit-forming microorganisms.

3. A process for refining distillate fuel oil comprising providing at least two fuel oil fractions boiling in the No. 2 fuel oil range, one of said fractions possessing a total acid number above about 0.1 and the other of said fractions possessing a total acid number not greater than about 0.1, subjecting at least a portion of the fraction that has a total acid number above about 0.1 to an additional refining treatment involving first, intimate contact thereof with about 2 to 20 percent by volume of about 2° to 40° Bé aqueous caustic soda solution, separating the neutralized fuel oil fraction from the partially spent caustic soda solution, and then water-washing the oil with about 10 to 200 volume percent wash-water to remove water-soluble materials from the treated oil, wherein the water used in at least one of said aqueous refining agent and said water-washing contains fuel oil gel deposit-forming microorganisms, and prior to said water-washing, incorporating in the wash-water, in a microbicidal proportion of about 0.005 to 0.05 percent,

the sodium salt of 2,4,5-trichlorophenol, and after separation of the washed, neutralized oil from wash-water, blending the washed, neutralized oil with the fuel oil fraction that has a total acid number of not greater than about 0.1, to form a blended distillate fuel oil that has a total acid number of not greater than about 0.1 and that has a reduced tendency to deposit gel due to gel deposit-forming microorganisms.

References Cited in the file of this patent

UNITED STATES PATENTS

|           |                |               |
|-----------|----------------|---------------|
| 1,991,329 | Mills          | Feb. 12, 1935 |
| 2,608,522 | Niehaus et al. | Aug. 26, 1952 |
| 2,680,058 | Harris et al.  | June 1, 1954  |

OTHER REFERENCES

Frear: "A Catalogue of Insecticides and Fungicides," 1948, vol. 2, page 42.

Reprint from Bacteriological Reviews, vol. 18, No. 4, December 1954, "Microbiology in the Petroleum Industry," by Davis et al., pages 230 and 233 (complete article, pages 215-238).